



US005466569A

**United States Patent** [19]**Weber et al.**[11] **Patent Number:** **5,466,569**[45] **Date of Patent:** **Nov. 14, 1995**[54] **COLOUR PHOTOGRAPHIC RECORDING MATERIAL**[75] Inventors: **Beate Weber**, Leichlingen; **Jörg Hagemann**, Köln; **Markus Geiger**, Langenfeld, all of Germany[73] Assignee: **Agfa-Gevaert AG**, Leverkusen, Germany[21] Appl. No.: **257,532**[22] Filed: **Jun. 9, 1994**[30] **Foreign Application Priority Data**

Jun. 21, 1993 [DE] Germany ..... 43 20 444.9

[51] Int. Cl.<sup>6</sup> ..... **G03C 1/08**; G03C 7/26; G03C 7/32[52] U.S. Cl. ..... **430/551**; 430/502; 430/557; 430/567; 430/372[58] **Field of Search** ..... 430/551, 372, 430/502, 557, 567, 505[56] **References Cited**

## U.S. PATENT DOCUMENTS

- 3,632,631 1/1972 Wright ..... 560/133  
 3,700,455 10/1972 Ishikawa et al. ..... 96/100  
 4,230,857 10/1980 Drake et al. ..... 544/388  
 5,098,477 3/1992 Vieira et al. ..... 106/22  
 5,294,530 3/1994 Seto et al. ..... 430/551

## FOREIGN PATENT DOCUMENTS

- 0246766 11/1987 European Pat. Off. .  
 0362604 4/1990 European Pat. Off. .  
 0373574 6/1990 European Pat. Off. .  
 2392000 12/1978 France .  
 251850 8/1986 Japan .

## OTHER PUBLICATIONS

Patent Abstracts of Japan, vol. 11, No. 103 (p. 562).

*Primary Examiner*—Charles L. Bowers, Jr.  
*Assistant Examiner*—Geraldine Letscher  
*Attorney, Agent, or Firm*—Connolly & Hutz[57] **ABSTRACT**

A color photographic material, at least one layer of which contains a compound of the formula (I)



in which

X means —NH—, —NR— or —O—,

R means alkyl, cycloalkyl or aryl,

R<sub>1</sub> means a chemical bond or a divalent bridging member, R<sub>2</sub> and R<sub>3</sub> mean alkyl, alkoxy, alkenyl, cycloalkyl, aryl or aryloxy, or two residues R<sub>2</sub> or R<sub>3</sub> mean the remaining atoms of a benzene ring condensed with the phenyl residue andm and n mean 0 to 3, wherein all alkyl, alkoxy, cycloalkyl, alkenyl, aryl and aryloxy residues may be further substituted and in each of the two phenyl residues a residue R<sub>1</sub>, R<sub>2</sub> or R<sub>3</sub> is in para position relative to the oxygen atom, is characterized by improved dye stability after processing.**5 Claims, No Drawings**

COLOUR PHOTOGRAPHIC RECORDING  
MATERIAL

The invention relates to a colour photographic recording material with improved dye stability.

Colour photographic materials customarily contain at least one yellow coupler, at least one magenta coupler and at least one cyan coupler, from which the corresponding dyes are produced by exposure and development. These dyes, particularly those dyes constantly exposed to light, should have elevated colour stability, wherein particular value is attached to all three colours having colour stability which is as far as possible equally good so that in the event of slight fading, no colour distortion occurs.

In particular, yellow dyes produced from couplers with an open-chain ketomethylene grouping must be stabilised both against light and against dark-fading.

It has already been proposed in U.S. Pat. No. 3,700,455 to achieve this object with bisphenol compounds as stabilisers. The effect achieved with them is, however, still inadequate.

It has now surprisingly been found that very specific bisphenols may achieve this object much more effectively.

The present invention thus provides a colour photographic material which contains on a support at least one blue-sensitive silver halide emulsion layer containing at least one yellow coupler, at least one green-sensitive silver halide emulsion layer containing at least one magenta coupler, at least one red-sensitive silver halide emulsion layer containing at least one cyan coupler, together with customary non-light-sensitive layers, characterised in that at least one layer contains a compound of the formula (I)



35

40

45

in which

X means —NH—, —NR— or —O—,

R means alkyl, cycloalkyl or aryl,

R<sub>1</sub> means a chemical bond or a divalent bridging member,

R<sub>2</sub> and R<sub>3</sub> mean alkyl, alkoxy, alkenyl, cycloalkyl, aryl or aryloxy, or two residues R<sub>2</sub> or R<sub>3</sub> mean the remaining atoms of a benzene ring condensed with the phenyl residue and

m and n mean 0 to 3, wherein all alkyl, alkoxy, cycloalkyl, alkenyl, aryl and aryloxy residues may be further substituted and in each of the two phenyl residues a residue R<sub>1</sub>, R<sub>2</sub> or R<sub>3</sub> is in para position relative to the oxygen atom.

Suitable bridging members R<sub>1</sub> are, for example alkene, alkylidene or sulphonyl groups together with heteroatoms such as O and S. Examples of R are methyl, ethyl, propyl, tert.-butyl, n-butyl, cyclohexyl, dodecyl, hexadecyl and benzyl.

Preferred compounds of the formula (I) are those of the formula (II)



in which

X means —NH—, —O— or —NR—

R<sub>4</sub>, R<sub>5</sub>, R<sub>7</sub> and R<sub>8</sub> mean alkyl or aryl,

R<sub>6</sub> means alkyl, cyclohexyl, acryloxyethyl or methacryloxyethyl.

R and R<sub>1</sub> have the above-stated meaning and the alkyl and aryl residues may be further substituted.

Suitable compounds of the formula I are:

| No.  | R <sub>1</sub>                       | R <sub>4</sub> /R <sub>7</sub>   | R <sub>5</sub> /R <sub>8</sub>  | X                                  | R <sub>6</sub>                                          |
|------|--------------------------------------|----------------------------------|---------------------------------|------------------------------------|---------------------------------------------------------|
| I-1  | CH <sub>2</sub>                      | CH <sub>3</sub>                  | CH <sub>3</sub>                 | N                                  | C <sub>12</sub> H <sub>25</sub>                         |
| I-2  | CH <sub>2</sub>                      | t-C <sub>4</sub> H <sub>9</sub>  | CH <sub>3</sub>                 | NH                                 | Cyclohexyl                                              |
| I-3  | CH <sub>2</sub>                      | t-C <sub>4</sub> H <sub>9</sub>  | CH <sub>3</sub>                 | NH                                 | Phenyl                                                  |
| I-4  | CH <sub>2</sub>                      | t-C <sub>4</sub> H <sub>9</sub>  | CH <sub>3</sub>                 | NH                                 | C <sub>12</sub> H <sub>25</sub>                         |
| I-5  | CH <sub>2</sub>                      | Cyclohexyl                       | CH <sub>3</sub>                 | NH                                 | C <sub>12</sub> H <sub>25</sub>                         |
| I-6  | CH <sub>2</sub>                      | t-C <sub>4</sub> H <sub>9</sub>  | CH <sub>3</sub>                 | NH                                 | CH <sub>2</sub> —CH <sub>2</sub> OCOCH=CH <sub>2</sub>  |
| I-7  | CH <sub>2</sub>                      | t-C <sub>4</sub> H <sub>11</sub> | CH <sub>3</sub>                 | NH                                 | CH <sub>2</sub> —CH <sub>2</sub> —OCOCH=CH <sub>2</sub> |
| I-8  | CH <sub>2</sub>                      | t-C <sub>5</sub> H <sub>11</sub> | CH <sub>3</sub>                 | NH                                 | C <sub>12</sub> H <sub>25</sub>                         |
| I-9  | CH <sub>2</sub>                      | t-C <sub>4</sub> H <sub>9</sub>  | t-C <sub>4</sub> H <sub>9</sub> | NH                                 | C <sub>12</sub> H <sub>25</sub>                         |
| I-10 | CH(C <sub>3</sub> H <sub>7</sub> )   | t-C <sub>4</sub> H <sub>9</sub>  | CH <sub>3</sub>                 | NH                                 | Phenyl                                                  |
| I-11 | CH <sub>2</sub>                      | t-C <sub>4</sub> H <sub>9</sub>  | n-C <sub>4</sub> H <sub>9</sub> | NH                                 | C <sub>12</sub> H <sub>25</sub>                         |
| I-12 | CH(C <sub>3</sub> H <sub>7</sub> )   | Cyclohexyl                       | CH <sub>3</sub>                 | NH                                 | Cyclohexyl                                              |
| I-13 | CH(C <sub>3</sub> H <sub>7</sub> )   | t-C <sub>4</sub> H <sub>9</sub>  | CH <sub>3</sub>                 | NH                                 | CH <sub>2</sub> —CH <sub>2</sub> —OCOCH=CH <sub>2</sub> |
| I-14 | CH <sub>2</sub>                      | Cyclohexyl                       | CH <sub>3</sub>                 | NH                                 | Cyclohexyl                                              |
| I-15 | CH <sub>2</sub>                      | t-C <sub>4</sub> H <sub>9</sub>  | CH <sub>3</sub>                 | N(CH <sub>3</sub> )                | Phenyl                                                  |
| I-16 | CH(i-C <sub>3</sub> H <sub>7</sub> ) | CH <sub>3</sub>                  | CH <sub>3</sub>                 | N(CH <sub>3</sub> H <sub>9</sub> ) | C <sub>4</sub> H <sub>9</sub>                           |
| I-17 | CH <sub>2</sub>                      | t-C <sub>4</sub> H <sub>9</sub>  | t-C <sub>4</sub> H <sub>9</sub> | N(CH <sub>3</sub> )                | CH <sub>2</sub> —CH <sub>2</sub> OCOCH=CH <sub>2</sub>  |
| I-18 |                                      | t-C <sub>4</sub> H <sub>9</sub>  | CH <sub>3</sub>                 | O                                  | C <sub>2</sub> H <sub>5</sub>                           |

-continued

| No.  | R <sub>1</sub>                         | R <sub>4</sub> /R <sub>7</sub>   | R <sub>5</sub> /R <sub>8</sub>   | X                                 | R <sub>6</sub>                   |
|------|----------------------------------------|----------------------------------|----------------------------------|-----------------------------------|----------------------------------|
| I-19 | CH <sub>2</sub>                        | t-C <sub>4</sub> H <sub>9</sub>  | t-C <sub>4</sub> H <sub>9</sub>  | O                                 | C <sub>4</sub> H <sub>9</sub>    |
| I-20 | CH <sub>2</sub>                        | t-C <sub>4</sub> H <sub>9</sub>  | C <sub>2</sub> H <sub>5</sub>    | O                                 | C <sub>16</sub> H <sub>33</sub>  |
| I-21 | CH <sub>2</sub>                        | t-C <sub>4</sub> H <sub>9</sub>  | CH <sub>3</sub>                  | O                                 | C <sub>2</sub> H <sub>5</sub>    |
| I-22 | CH <sub>2</sub>                        | 1-Methyl-cyclohexyl              | CH <sub>3</sub>                  | O                                 | C <sub>2</sub> H <sub>5</sub>    |
| I-23 | CH <sub>2</sub>                        | Cyclohexyl                       | CH <sub>3</sub>                  | O                                 | C <sub>4</sub> H <sub>9</sub>    |
| I-24 |                                        | CH <sub>3</sub>                  | CH <sub>3</sub>                  | O                                 | C <sub>16</sub> H <sub>33</sub>  |
|      |                                        |                                  |                                  |                                   |                                  |
| I-25 | CH(iso-C <sub>3</sub> H <sub>7</sub> ) | CH <sub>3</sub>                  | CH <sub>3</sub>                  | O                                 | C <sub>2</sub> H <sub>5</sub>    |
| I-26 | CH(t-C <sub>4</sub> H <sub>9</sub> )   | CH <sub>3</sub>                  | CH <sub>3</sub>                  | O                                 | CH <sub>2</sub> CCl <sub>3</sub> |
| I-27 | S                                      | t-C <sub>4</sub> H <sub>9</sub>  | CH <sub>3</sub>                  | O                                 | C <sub>16</sub> H <sub>33</sub>  |
| I-28 | S                                      | t-C <sub>4</sub> H <sub>9</sub>  | CH <sub>3</sub>                  | N(C <sub>4</sub> H <sub>9</sub> ) | C <sub>4</sub> H <sub>9</sub>    |
| I-29 | O                                      | t-C <sub>5</sub> H <sub>11</sub> | t-C <sub>5</sub> H <sub>11</sub> | NH                                | t-C <sub>4</sub> H <sub>9</sub>  |
| I-30 |                                        |                                  |                                  |                                   |                                  |
| I-31 |                                        |                                  |                                  |                                   |                                  |
| I-32 |                                        |                                  |                                  |                                   |                                  |
| I-33 |                                        |                                  |                                  |                                   |                                  |
| I-34 |                                        |                                  |                                  |                                   |                                  |

-continued

| No.  | R <sub>1</sub> | R <sub>4</sub> /R <sub>7</sub> | R <sub>5</sub> /R <sub>8</sub> | X | R <sub>6</sub> |
|------|----------------|--------------------------------|--------------------------------|---|----------------|
| I-35 |                |                                |                                |   |                |
| I-36 |                |                                |                                |   |                |
| I-37 |                |                                |                                |   |                |
| I-38 |                |                                |                                |   |                |

The compounds are preferably used in a layer containing 55 colour couplers in a quantity of 0.1 to 2 mol/mol of colour coupler, in particular in a quantity of 0.1 to 0.5 mol/mol of colour coupler.

In a preferred embodiment, the compounds of the formulae I or II are used in combination with other colour stabilisers, wherein compounds of the formulae III, IV and V below may be considered as further colour stabilisers, which are preferably used in a layer containing a colour 60 coupler in a quantity of 0.05 to 2 mol/mol of colour coupler, in particular 0.05 to 0.5 mol/mol of colour coupler. 65



with

Y=a residue which may be cleaved under chromogenic development conditions, for example acyl, R<sup>31</sup>=alkyl, cycloalkyl, acylamino, sulphonamino,

7

$R^{32}$ ,  $R^{33}$ ,  $R^{34}=H$  alkyl cycloalkyl, hydroxy, acyloxy, alkoxy carbonyl, halogen, acylamino, carbamoyl,  $R^{35}=\text{alkyl, cycloalkyl, alkoxy carbonyl, acylamino, carbamoyl.}$

Two adjacent residues R<sup>31</sup> to R<sup>35</sup> may form a 5- or 5-6-membered ring.



with

$R^{41}$ =H, OH, alkoxy, aryloxy, acyl, acyloxy, alkyl, cycloalkyl. 15

$R^{42}, R^{43} \equiv H$  alkyl

$R^4, R^5 = H, \text{alkyl}$

$R'$ ,  $R$  = *alkyl*, *cycloalkyl*,  
 $Z$ =a group to complete a non-metallic 5- to 8-membered ring

The residues  $R^{42}$  and  $R^{45}$ ,  $R^{43}$  and  $R^{44}$ ,  $R^{41}$  and  $R^{44}$  or  $R^{45}$  may form a 5- to 8-membered ring. 20

IV

10

$$\text{R}^{51}-\text{S}-\text{R}^{\uparrow}$$

V

with

$R^{51}, R^{52}$ =alkyl, cycloalkyl, aryl.

The residues  $R^{51}$  and  $R^{52}$  may also form a 5- to 8-membered ring

The alkyl or aryl residues may be substituted, for example with hydroxyl, alkyl, aryl, hetaryl, alkoxy, aryloxy, acyloxy, alkoxy carbonyl, acylamino, carbamoyl, sulphonamino, sulphamoyl, sulphonyl and halogen.

An acyl residue may be derived from a carboxylic acid (for example acetyl, acrylic), a carbamic acid (for example dodecylaminocarbonyl, butylaminocarbonyl) or a carbonic acid semi-ester (for example ethoxycarbonyl, hexyldeoxycarbonyl).

Compounds III, IV and V may also be linked to a polymer chain by one of the substituents.

Examples of compounds of the formulae III, IV and V are



-continued



The compounds according to the invention are preferably used in combination with yellow couplers. Colour stabilisation of the photographic materials is, however, also achieved with other couplers, magenta and cyan couplers. 60 Yellow couplers are preferably used in a quantity of 0.1 to 1 mmol/m<sup>2</sup> of material.

#### Synthesis of compound I-4

6.8 g of 2,2'-methylene-bis(6-tert-butyl-4-methylphenol) in 30 ml of acetone are stirred overnight at room 65 temperature with 4.42 g of dodecyl isocyanate. The solution is poured into H<sub>2</sub>O, the precipitate filtered out, washed with

water and dried under a vacuum at 40° C. The product is stirred with methanol to purify it further.

Yield: 55% Melting point: 112°–116° C.

#### Synthesis of compound I-6

6.8 g of 2,2'-methylene-bis(6-tert-butyl-4-methylphenol) in 30 ml of acetone are stirred overnight at room temperature with 3.1 g of isocyanatoethyl methacrylate. The solution is poured into H<sub>2</sub>O, the residue stirred with H<sub>2</sub>O and dried under a vacuum at 40° C. The solid is recrystallised from hexane.

Yield: 69% Melting point: 138°–142° C.

## Synthesis of compound I-21

2.17 g of ethyl chloroformate are added dropwise at 0°C. to 6.8 g of 2,2'-methylene-bis-(6-tert.-butyl-4-methylphenol) and 2.02 g of triethylamine in 10 ml of acetone. The reaction solution is stirred for 4 hours at room temperature and then mixed with H<sub>2</sub>O. The residue is filtered out and recrystallised from ethanol.

Yield: 85% Melting point: 129°–130°C.

The yellow couplers, which are preferably used in a single layer with dye stabilisers according to the invention, are preferably 2-equivalent pivaloyl yellow couplers, the leaving group of which is attached to the coupling position of the coupler either with oxygen or with nitrogen.

Suitable yellow couplers are:



Y-1: R<sup>1</sup> = —C<sub>4</sub>H<sub>9</sub>-t;



R<sup>3</sup> = Cl;

R<sup>4</sup> = H;



Y-2: R<sup>1</sup> = —C<sub>4</sub>H<sub>9</sub>-t;



R<sup>3</sup> = —OC<sub>16</sub>H<sub>33</sub>;

R<sup>4</sup> = H;

R<sup>5</sup> = —SO<sub>2</sub>NHCH<sub>3</sub>

Y-3: R<sup>1</sup> = —C<sub>4</sub>H<sub>9</sub>-t;



R<sup>3</sup> = Cl;

R<sup>4</sup> = H;

R<sup>5</sup> = —NHSO<sub>2</sub>—C<sub>16</sub>H<sub>33</sub>

Y-4: R<sup>1</sup> = —C<sub>4</sub>H<sub>9</sub>-t;

-continued



5

R<sup>3</sup> = Cl;

R<sup>4</sup> = H;

R<sup>5</sup> = —COOC<sub>12</sub>H<sub>25</sub>

10

Y-5: R<sup>1</sup> = —C<sub>4</sub>H<sub>9</sub>-t;



20

R<sup>3</sup> = Cl;

R<sup>4</sup> = H;



25

Y-6: R<sup>1</sup> = —C<sub>4</sub>H<sub>9</sub>-t;



30

R<sup>3</sup> = Cl;

R<sup>4</sup> = H;



35

Y-7: R<sup>1</sup> = —C<sub>4</sub>H<sub>9</sub>-t;



40

R<sup>3</sup> = Cl;

R<sup>4</sup> = H;

R<sup>5</sup> = —NHSO<sub>2</sub>—C<sub>16</sub>H<sub>33</sub>

45

Y-8: R<sup>1</sup> = —C<sub>4</sub>H<sub>9</sub>-t;



50

R<sup>3</sup> = Cl;

R<sup>4</sup> = H;

R<sup>5</sup> = —CH(CH<sub>3</sub>)<sub>2</sub>

55

R<sup>3</sup> = Cl;

-continued

 $R^4 = H;$ Y-9:  $R^1 = -\text{C}_4\text{H}_9-t;$  $R^3 = -\text{OC}_{16}\text{H}_{33};$  $R^4 = H;$  $R^5 = -\text{SO}_2\text{NHCO}_2\text{C}_2\text{H}_5$ Y-10:  $R^1 = -\text{C}_4\text{H}_9-t;$  $R^3 = \text{Cl};$  $R^4 = H$ Y-11:  $R^1 = -\text{C}_4\text{H}_9-t;$  $R^3 = \text{Cl};$  $R^4 = H;$ Y-12:  $R^1 = -\text{C}_4\text{H}_9-t;$  $R^3 = \text{Cl};$ 

-continued

 $R^4 = H;$ 

5

10 Y-13:  $R^1 = -\text{C}_4\text{H}_9-t;$  $R^3 = -\text{OC}_{16}\text{H}_{33};$ 20  $R^4 = H;$  $R^5 = -\text{SO}_2\text{NHCH}_3$ Y-14:  $R^1 = -\text{C}_4\text{H}_9-t;$  $R^3 = \text{Cl};$ 30  $R^4 = H;$  $R^2, R^4, R^5 = H;$ 50  $R^3 = -\text{OCH}_3$ 65  $R^3, R^5 = -\text{OCH}_3;$

-continued

 $R^4 = H$  $R^4 = OCH_3;$  $R^5 = H;$  $R^6 = -SO_2N(CH_3)_2$ 

-continued

 $R^4 = H;$ 

5

10 Y-21:  $R_1 = t-C_4H_9$ 15  $R_3 = OCH_3;$ 20  $R_4 = H.$ 

25  $R_5 = NHCOCH(CH_3)CH_2-SO_2-C_{12}H_{25}$

Y-22:  $CH_3O-$

$COCH-$

$CONH-$

$OC_2H_5$

$CH_3$

$OC_2H_5$

$CH_3$

Y-23:

$N-COCH_2-$

$CONH-$

$Cl$

45  $SO_2NHCONHC_{12}H_{25}(n)$

Y-24:

$CH_3$

$CO-CH-$

$CONH-$

$OC_{16}H_{33}(n)$

$SO_2NHCO-N$

50  $CH_3$

55

60

-continued



The support may be reflective or transparent.

Silver halides which may be considered for the silver halide layers containing colour couplers and those not containing colour couplers are AgBr, AgBrCl, AgBrClI and AgCl.

Preferably, the silver halides of all the light-sensitive layers, including the interlayers according to the invention, contain at least 80 mol % chloride, in particular 95 to 100 mol % chloride, 0 to 5 mol % bromide and 0 to 1 mol % iodide. The silver halide emulsions may be directly positive or preferably negative emulsions.

The silver halide crystals may be predominantly compact, for example regularly cubic or octahedral or they may have transitional shapes. Preferably, however, twinned, for example lamellar, crystals may also be present, the average ratio of diameter to thickness of which is preferably at least 5:1, wherein the diameter of a grain is defined as the diameter of a circle the contents of which correspond to the projected surface area of the grain. The layers may, however, also have tabular silver halide crystals, in which the ratio of diameter to thickness is greater than 5:1, for example 12:1 to 30:1.

The silver halide grains may also have a multi-layered grain structure, in the simplest case with one internal zone and one external zone of the grain (core/shell), wherein the halide composition and/or other modifications, such as for example doping, of the individual grain zones are different. The average grain size of the emulsions is preferably between 0.2  $\mu\text{m}$  and 2.0  $\mu\text{m}$ , the grain size distribution may be both homodisperse and heterodisperse. The emulsions may, in addition to the silver halide, also contain organic silver salts, for example silver benzotriazolate or silver behenate.

Two or more types of silver halide emulsions which are produced separately may be used as a mixture.

The photographic emulsions may be produced by various methods (for example P. Glafkides, *Chimie et Physique Photographique*, Paul Montel, Paris (1967), G. F. Duffin, *Photographic Emulsion Chemistry*, The Focal Press, London (1966), V. L. Zelikman et al, *Making and Coating Photographic Emulsion*, The Focal Press, London (1966)) from soluble silver salts and soluble halides.

Gelatine is preferably used as the binder. Gelatine may, however, be entirely or partially replaced with other synthetic, semi-synthetic or also naturally occurring polymers.

The binders should have a sufficient quantity of functional groups available so that satisfactorily resistant layers may be

produced by reaction with suitable hardeners. Such functional groups are in particular amino groups, but also carboxyl groups, hydroxyl groups and active methylene groups.

The photographic emulsions may contain compounds to prevent fogging or to stabilise the photographic function during production, storage or photographic processing.

Particularly suitable are azaindenes, preferably tetra- and pentazaindenes, particularly those substituted with hydroxyl or amino groups. Such compounds have been described, for example, by Birr, *Z. Wiss. Phot.*, 47, (1952), pages 2-58. Furthermore, salts of metals such as mercury or cadmium, aromatic sulphonic or sulphonic acids such as benzenesulphonic acid, or heterocyclics containing nitrogen such as nitrobenzimidazole, nitroindazole, (substituted) benzotriazoles or benzothiazolium salts may also be used as anti-fogging agents. Particularly suitable are heterocyclics containing mercapto groups, for example mercaptobenzothiazoles, mercaptobenzimidazoles, mercaptotetrazoles, mercaptodiimidazoles, mercaptopyrimidines, wherein these mercaptoazoles may also contain a water solubilising group, for example a carboxyl group or sulpho group. Further suitable compounds are published in *Research Disclosure* 17643 (December 1978), section VI.

The stabilisers may be added to the silver halide emulsions before, during or after ripening of the emulsions. Naturally, the compounds may also be added to other photographic layers which are assigned to a silver halide layer.

Mixtures of two or more of the stated compounds may also be used.

The silver halide emulsions are customarily chemically ripened, for example under the action of gold compounds or compounds of divalent sulphur.

The photographic emulsion layers or other hydrophilic colloidal layers of the light-sensitive material produced according to the invention may contain surface-active agents for various purposes, such as coating auxiliaries, to prevent formation of electric charges, to improve sliding properties, to emulsify the dispersion, to prevent adhesion and to improve photographic characteristics (e.g. acceleration of development, greater contrast, sensitisation etc.).

Cyanine dyes are suitable sensitising dyes, in particular those of the following classes:

1. Red sensitisers Dicarbocyanines with naphthothiazole or benzothiazole as basic terminal groups, which may be substituted in 5th and/or 6th position with halogen, methyl, methoxy, together with 9,11-alkene-bridged, in particular 9,11-neopentylidenethiadcarbocyanines with alkyl or sulphonyl substituents on the nitrogen.

2. Green sensitisers 9-ethyloxacarbocyanines, which are substituted in 5th position with chlorine or phenyl and which bear alkyl or sulphonyl residues, preferably sulphonyl substituents on the nitrogen of the benzoxazole groups.

3. Blue sensitisers Methinecyanines with benzoxazole, benzothiazole, benzoselenazole, naphthoxazole, naphthothiazole as basic terminal groups, which may be substituted in 5th and/or 6th position with halogen, methyl, methoxy and which bear at least one, preferably two, sulphonyl substituents on the nitrogen. Additionally, apomerocyanines with a rhodanine group.

Sensitisers may be dispensed with if the intrinsic sensitivity of the silver halide is sufficient for a specific spectral range, for example the blue sensitivity of silver bromide-iodides.

To the differently sensitised emulsion layers are assigned non-diffusing monomeric or polymeric colour couplers which may be located in the same layer or in an adjacent layer.

Usually, cyan couplers are assigned to the red-sensitive layers, magenta couplers to the green-sensitive layers and yellow couplers to the blue-sensitive layers.

Colour couplers to produce the cyan partial colour image are generally couplers of the phenol or  $\alpha$ -naphthol type.

Colour couplers to produce the magenta partial colour image are generally couplers of the pyrazoloazole, 5-pyrazolone, or indazolone type.

Colour couplers to produce the yellow partial colour image are generally couplers with an open-chain ketomethylene grouping, in particular couplers of the  $\alpha$ -acylacetamide type; suitable examples of which are  $\alpha$ -benzoylacetamide couplers and  $\alpha$ -pivaloylacetanilide couplers. As already mentioned, the latter are preferred.

The colour couplers may be 4-equivalent couplers, but they may also be 2-equivalent couplers. The latter are differentiated from 4-equivalent couplers by containing a substituent at the coupling position which is eliminated on coupling.

The couplers customarily contain a ballast residue in order to render diffusion within the material, i.e. both within a layer and between layers, impossible. High molecular weight couplers may also be used instead of couplers with a ballast residue.

Suitable colour couplers or references in which they are described may be found in *Research Disclosure* 17643 (1978), section VII.

High molecular weight colour couplers are, for example, described in DE-C-1 297 417, DE-A-24 07 569, DE-A-31 48 125, DE-A-32 17 200, DE-A-33 20 079, DE-A-33 24 932, DE-A-33 31 743, DE-A-33 40 376, EP-A-27 284, U.S. Pat. No. 4,080,211. The high molecular weight colour couplers are generally produced by polymerisation of ethylenically unsaturated monomeric colour couplers. They may, however, also be produced by polyaddition or polycondensation.

The incorporation of couplers or other compounds into the silver halide emulsion layers may proceed by initially producing a solution, dispersion or emulsion of the compound concerned and then adding it to the pouring solution for the layer concerned. Selection of the appropriate solvent or dispersant depends on the particular solubility of the compound.

Methods for the introduction of compounds which are essentially insoluble in water by a grinding process are described, for example, in DE-A-26 09 741 and DE-A-26 09 742.

Hydrophobic compounds may also be introduced into the pouring solution by using high-boiling solvents, so-called oil formers. Corresponding methods are described, for example, in U.S. Pat. Nos. 2,322,027, 2,801,170, 2,801,171 and EP-A-0 043 037.

Instead of high-boiling solvents, oligomers or polymers, so-called polymeric oil formers, may be used.

The compounds may also be introduced into the pouring solution in the form of filled latices. Reference is, for example, made to DE-A-25 41 230, DE-A-25 41 274, DE-A-28 35 856, EP-A-0 014 921, EP-A-0 069 671, EP-A-0 130 115, U.S. Pat. No. 4,291,113.

The non-diffusible inclusion of anionic water-soluble compounds (for example of dyes) may also proceed with the assistance of cationic polymers, so-called mordanting polymers.

Suitable oil formers are, for example, phthalic acid alkyl esters, phosphonic acid esters, phosphoric acid esters, citric acid esters, benzoic acid esters, amides, fatty acid esters, trimesic acid esters, alcohols, phenols, aniline derivatives, hydrocarbons, sulphones and sulphoxides.

Examples of suitable oil formers are dibutyl phthalate, dicyclohexyl phthalate, di-2-ethylhexyl phthalate, decyl phthalate, triphenyl phosphate, tricresyl phosphate, 2-ethylhexyl diphenyl phosphate, tricyclohexyl phosphate, tri-2-ethylhexyl phosphate, tridecyl phosphate, tributoxyethyl phosphate, trichloropropyl phosphate, di-2-ethylhexylphenyl phosphate, 2-ethylhexyl benzoate, dodecyl benzoate, 2-ethylhexyl-p-hydroxybenzoate, diethyl dodecanamide, N-tetradecylpyrrolidone, isostearyl alcohol, 2,4-di-tert-amylophenol, dioctyl acetate, glycerol tributylate, iso-stearyl lactate, trioctyl citrate, N,N-dibutyl-2-butoxy-5-tert.-octyl aniline, paraffin, dodecylbenzene and diisopropyl naphthalene.

The photographic material may also contain UV light absorbing compounds, optical whiteners, spacers, filter dyes, formalin scavengers, light stabilisers, anti-oxidants,  $D_{min}$  dyes, additives to improve stabilisation of dyes, couplers and whites and to reduce colour fogging, plasticisers (latices), biocides and others. Interlayers may additionally contain so-called white couplers and other compounds which react with the developer oxidation product (scavengers).

The layers of the photographic material may be hardened with customary hardeners. Suitable hardeners are, for example, formaldehyde, glutaraldehyde and similar aldehyde compounds, diacetyl, cyclopentadione and similar ketone compounds, bis-(2-chloroethylurea), 2-hydroxy-4,6-dichloro-1,3,5-triazine and other compounds containing reactive halogen (U.S. Pat. Nos. 3,288,775, 2,732,303, GB-A-974 723 and GB-A-1 167 207), divinylsulphone compounds, 5-acetyl-1,3-diacryloylhexahydro-1,3,5-triazine and other compounds containing a reactive olefin bond (U.S. Pat. Nos. 3,635,718, 3,232,763 and GB-A-994 869); N-hydroxymethylphthalimide and other N-methylol compounds (U.S. Pat. Nos. 2,732,316 and 2,586,168); isocyanates (U.S. Pat. No. 3,103,437); aziridine compounds (U.S. Pat. Nos. 3,017,280 and 2,983,611); acid derivatives (U.S. Pat. Nos. 2,725,294 and 2,725,295); compounds of the carbodiimide type (U.S. Pat. No. 3,100,704); carbamoylpyridinium salts (DE-A-22 25 230 and DE-A-24 39 551); carbamoyloxy pyridinium compounds (DE-A-24 08 814); compounds with a phosphorus-halogen bond (JP-A-113 929/83); N-carboxyloximide compounds (JP-A-43353/81); N-sulphonyloximido compounds (U.S. Pat. No. 4,111,926), dihydroquinoline compounds (U.S. Pat. No. 4,013,468), 2-sulphonyloxy pyridinium salts (JP-A-110 762/81), formamidinium salts (EP-A-0 162 308), compounds with two or more N-acyloximino groups (U.S. Pat. No. 4,052,373), epoxy compounds (U.S. Pat. No. 3,091,537), compounds of the isoxazole type (U.S. Pat. Nos. 3,321,313 and 3,543,292); halogen carboxyaldehydes, such as mucochloric acid; dioxane derivatives, such as dihydroxydioxane and dichlorodioxane; and inorganic hardeners such as chrome alum and zirconium sulphate.

Hardening may be effected in a known manner by adding the hardener to the pouring solution for the layer to be hardened, or by overcoating the layer to be hardened with a layer containing a diffusible hardener.

There are included in the classes listed, slow acting and fast acting hardeners as well as so-called instant hardeners, which are particularly advantageous. Instant hardeners are understood to be compounds which crosslink suitable binders in such a way that immediately after pouring, at the latest after 24 hours, preferably at the latest after 8 hours, hardening is concluded to such an extent that there is no further alteration in the sensitometry and swelling of the layered structure determined by the crosslinking reaction. Swelling

is understood as the difference between the wet layer thickness and the dry layer thickness during aqueous processing of the film (*Photogr. Sci. Eng.* 8 (1964), 275; *Photogr. Sci. Eng.* (1972), 449).

These hardeners which react very rapidly with gelatine are, for example, carbamoylpyridinium salts, which are capable of reacting with the free carboxyl groups of the gelatine, so that the latter react with free amino groups of the gelatine forming peptide bonds and crosslinking the gelatine.

There are diffusible hardeners which have the same hardening effect on all the layers in a layered structure. There are, however, also non-diffusing low molecular weight and high molecular weight hardeners the action of which is restricted within a layer. Using these, individual layers, for example the protective layer, may be particularly highly crosslinked. This is important if the silver halide layer is sparingly hardened in order to increase the silver covering power and the mechanical properties of the protective layer must be improved (EP-A-0 114 699).

The colour photographic materials according to the invention are customarily processed by developing, bleaching, fixing and rinsing or by developing, bleaching, fixing and stabilising without subsequent rinsing, wherein bleaching and fixing may be combined into a single processing stage. Colour developer compounds which may be used are all developer compounds having the ability to react, in the form of their oxidation product, with colour couplers to azomethine or indophenol dyes. Suitable colour developer compounds are aromatic compounds containing at least one primary amino group of the p-phenylenediamine type, for example N,N-dialkyl-p-phenylenediamines such as N,N-diethyl-p-phenylenediamine, 1-(N-ethyl-N-methanesulphonamidoethyl)-3-methyl-p-phenylenediamine, N-ethyl-N-3-hydroxypropyl-3-methyl-p-phenylenediamine and 1-(N-ethyl-N-methoxyethyl)-3-methyl-p-phenylenediamine. Further usable colour developers are described for example in *J. Amer. Chem. Soc.* 73, 3106 (1951) and G. Haist *Modern Photographic Processing*, 1979, John Wiley & Sons, New York, pages 545 et seq.

An acid stop bath or rinsing may follow after colour development.

Customarily, the material is bleached and fixed immediately after colour development. Bleaches which may be used are, for example, Fe(III) salts and Fe(III) complex salts such as ferricyanides, dichromates, water soluble cobalt complexes. Iron(III) complexes of aminopolycarboxylic acids are particularly preferred, in particular for example complexes of ethylenediaminetetraacetic acid, propylenediaminetetraacetic acid, diethylenetriaminepentaacetic acid, nitrilotriacetic acid, iminodiacetic acid, N-hydroxyethyl-ethylenediaminetriacetic acid, alkyliminodicarboxylic acids and of corresponding phosphonic acids. Persulphates and peroxides, for example hydrogen peroxide, are also suitable as bleaches.

Rinsing usually follows the bleaching-fixing bath or fixing bath, which is performed as countercurrent rinsing or consists of several tanks with their own water supply.

Favourable results may be obtained by using a subsequent finishing bath which contains no or only a little formaldehyde.

Rinsing may, however, be completely replaced with a stabilising bath, which is customarily performed countercurrently. If formaldehyde is added, this stabilising bath also performs the function of a finishing bath.

## EXAMPLE 1

The following two layers were applied to paper coated on both sides with polyethylene. The quantities relate in each case to one m<sup>2</sup>.

1st layer

Blue-sensitive silver halide emulsion layer prepared from 0.6 g AgNO<sub>3</sub>.

(99.5 mol % chloride, 0.5 mol % bromide, average grain diameter 0.78 µm).

2 g gelatine 0.8 g yellow coupler Y-9 0.6 g DBP Stabiliser according to table 1 in a quantity of 0.5 mol/mol of coupler

2nd layer

2 g gelatine 0.4 g hardener of formula



The samples were then exposed behind a graduated grey wedge and processed in the customary manner using the processing baths listed below.

a) Colour developer—45 sec-35° C.

|                                                                       |          |
|-----------------------------------------------------------------------|----------|
| Triethanolamine                                                       | 9.0 g/l  |
| N,N-diethylhydroxylamine                                              | 4.0 g/l  |
| Diethylene glycol                                                     | 0.05 g/l |
| 3-methyl-4-amino-N-ethyl-N-methane-sulphonaminoethyl-aniline sulphate | 5.0 g/l  |
| Potassium sulphite                                                    | 0.2 g/l  |
| Triethylene glycol                                                    | 0.05 g/l |
| Potassium carbonate                                                   | 22 g/l   |
| Potassium hydroxide                                                   | 0.4 g/l  |
| Ethylenediaminetetraacetic acid disodium salt                         | 2.2 g/l  |
| Potassium chloride                                                    | 2.5 g/l  |
| 1,2-dihydroxybenzene-3,4,6-trisulphonic acid trisodium salt           | 0.3 g/l  |
| make up to 1000 ml with water; pH 10.0                                |          |

b) Bleach fixing bath—45 sec-35° C.

|                                                      |          |
|------------------------------------------------------|----------|
| Ammonium thiosulphate                                | 75 g/l   |
| Sodium hydrogen sulphite                             | 13.5 g/l |
| Ammonium acetate                                     | 2.0 g/l  |
| Ethylenediaminetetraacetic acid (iron-ammonium salt) | 57 g/l   |
| Ammonia, 25 wt. %                                    | 9.5 g/l  |
| Acetic acid                                          | 9.0 g/l  |
| make up to 1000 ml with water; pH 5.5                |          |

c) Rinsing—2 min-35° C.

d) Drying

The processed samples are then covered with a UV protective film and exposed in a xenon test device to determine light-fastness (40% relative humidity; 25° C.; 19.2·10<sup>6</sup> lxh).

The UV protective film was produced as follows: a layer prepared from 1.5 g of gelatine, 0.65 g of UV absorber of the following formula



0.07 g of dioctylhydroquinone and 0.36 g of tricresyl phosphate was applied to a transparent cellulose triacetate film which had been provided with a coupling layer. The quantities relate to 1 m<sup>2</sup>.

TABLE 1

| Sample       | Stabiliser | Percentage reduction in density at density |     |                  |
|--------------|------------|--------------------------------------------|-----|------------------|
|              |            | 0.5                                        | 1.0 | D <sub>max</sub> |
| 1 Comparison | —          | 75                                         | 74  | 77               |
| 2 Comparison | X-1        | 63                                         | 57  | 53               |
| 3 Comparison | X-2        | 65                                         | 59  | 50               |
| 4 Comparison | X-3        | 62                                         | 56  | 49               |
| 5 Invention  | I-4        | 41                                         | 25  | 33               |
| 6 Invention  | I-6        | 44                                         | 26  | 37               |
| 7 Invention  | I-14       | 45                                         | 27  | 36               |
| 8 Invention  | I-21       | 46                                         | 27  | 37               |
| 9 Invention  | I-25       | 42                                         | 24  | 32               |

As table 1 shows, improved light stability of the yellow dyes is achieved with the compounds according to the invention, particularly at medium to high densities.



## EXAMPLE 2

A colour photographic recording material suitable for rapid processing was produced by applying the following layers in the stated sequence onto a film support coated on both sides with polyethylene. The quantities relate in each case to 1 m<sup>2</sup>. The corresponding quantities of AgNO<sub>3</sub> are stated for the quantity of silver halide applied.

Layer structure sample 1

Layer 1: (Substrate) 0.2 g gelatine

Layer 2: (Blue-sensitive layer) Blue-sensitive silver

halide emulsion (99.5 mol % chloride, 0.5 mol % bromide, average grain diameter 0.8 μm) prepared from 0.45 g AgNO<sub>3</sub> with 1.08 g gelatine 0.60 g yellow coupler Y-21 0.215 g white coupler W-1 0.30 g tricresyl phosphate (TCP)

5 Layer 3: (Protective layer) 1.1 g gelatine 0.06 g 2,5-dioctylhydroquinone 0.06 g dibutyl phthalate (DBP)

Layer 4: (Green-sensitive layer) Green-sensitised silver halide emulsion (99.5 mol % chloride, 0.5 mol % bromide, average grain diameter 0.6 μm) prepared from 0.45 g AgNO<sub>3</sub> with 1.08 g gelatine 0.41 g magenta coupler M-1 0.15 g image stabiliser ST-1 0.30 g image stabiliser ST-2 0.08 g 2,5-dioctylhydroquinone 0.34 g DBP 0.04 g TCP

10 Layer 5: (UV protective layer) 1.15 g gelatine 0.6 g UV absorber UV-1 0.045 g 2,5-dioctylhydroquinone 0.04 g TCP

Layer 6: (Red-sensitive layer) Red-sensitised silver halide emulsion (99.5 mol % chloride, 0.5 mol % bromide, average grain diameter 0.5 μm) prepared from 0.3 g AgNO<sub>3</sub> with 0.75 g gelatine 0.35 g cyan coupler C-1 0.36 g TCP

15 Layer 7: (UV protective layer) 0.35 g gelatine 0.15 g UV absorber UV-1 0.2 g TCP

Layer 8: (Protective layer) 0.9 g gelatine 0.3 g hardener H-1



## Samples 2 to 13

Samples 2 to 13 were produced in the same manner as sample 1, with the difference that 0.2 g/m<sup>2</sup> of a stabiliser as

stated in table 2 was added to layer 2.

In samples 9 to 13, 0.1 g/m<sup>2</sup> of a co-stabiliser of the formulae III, IV or V as stated in table 2 was additionally added to layer 2.

The samples were then exposed, processed and exposed to a xenon light source as in example 1. The measured percentage reductions in density are reproduced in table 2.

Exposed and processed samples were furthermore stored for 5 weeks in a heated cabinet at 80° C. and 50% relative humidity and fog and the percentage reduction in density at D<sub>max</sub> were then determined. The results are reproduced in table 3.

TABLE 2

| Sample    | Stabiliser | Co-stabiliser | Percentage reduction in density at density |     |     |
|-----------|------------|---------------|--------------------------------------------|-----|-----|
|           |            |               | 0.5                                        | 1.0 | 1.5 |
| 1 (comp.) | —          | —             | 55                                         | 30  | 42  |
| 2 (comp.) | X-1        | —             | 31                                         | 18  | 15  |
| 3 (comp.) | X-2        | —             | 52                                         | 25  | 22  |
| 4 (inv.)  | 1-4        | —             | 16                                         | 7   | 6   |
| 5 (inv.)  | 1-6        | —             | 18                                         | 9   | 8   |
| 6 (inv.)  | 1-14       | —             | 20                                         | 10  | 10  |
| 7 (inv.)  | 1-21       | —             | 21                                         | 10  | 11  |
| 8 (inv.)  | 1-25       | —             | 17                                         | 7   | 6   |
| 9 (comp.) | X-1        | III-4         | 28                                         | 17  | 14  |
| 10 (inv.) | 1-4        | III-4         | 13                                         | 5   | 4   |
| 11 (inv.) | 1-4        | V-2           | 12                                         | 5   | 4   |
| 12 (inv.) | 1-25       | IV-2          | 15                                         | 5   | 5   |
| 13 (inv.) | 1-25       | V-5           | 13                                         | 4   | 4   |

As is shown by table 2, the light stability of the yellow dye is distinctly improved by the compounds according to the invention in comparison with X-1 and X-2. Addition of co-stabilisers of the formulae III, IV and V makes it possible to improve light stability still further.

TABLE 3

| Sample    | yellow | magenta | cyan | % reduction in density |    |
|-----------|--------|---------|------|------------------------|----|
|           |        |         |      | 40                     | 45 |
| 1 (comp.) | 22     | 15      | 11   | 11                     |    |
| 2 (comp.) | 21     | 14      | 11   | 10                     |    |
| 3 (comp.) | 23     | 16      | 12   | 12                     |    |
| 4 (inv.)  | 16     | 12      | 10   | 6                      |    |
| 5 (inv.)  | 17     | 13      | 10   | 7                      |    |
| 6 (inv.)  | 18     | 13      | 10   | 7                      |    |
| 7 (inv.)  | 18     | 13      | 11   | 7                      |    |
| 8 (inv.)  | 17     | 12      | 10   | 6                      |    |
| 9 (comp.) | 21     | 14      | 11   | 10                     |    |
| 10 (inv.) | 15     | 12      | 20   | 5                      |    |
| 11 (inv.) | 13     | 10      | 8    | 3                      |    |
| 12 (inv.) | 16     | 12      | 9    | 6                      |    |
| 13 (inv.) | 13     | 10      | 9    | 3                      |    |

As is shown by table 3, dark-fading stability is improved by the compounds according to the invention. The compounds X-1 and X-2 used by way of comparison bring about a lesser improvement. Addition of compounds of the formulae III, IV and particularly V brings about a further improvement in dark-fading stability.

We claim:

1. A color photographic material which contains on a support at least one blue-sensitive silver halide emulsion layer containing at least one yellow coupler, at least one green-sensitive silver halide emulsion layer containing at least one magenta coupler, at least one red-sensitive silver halide emulsion layer containing at least one cyan coupler, at least one non-light-sensitive layer, characterised in that at least one layer contains a compound of the formula (II)



in which

R<sub>4</sub>, R<sub>5</sub>, R<sub>7</sub> and R<sub>8</sub> are the same or different and are alkyl, R<sub>6</sub> means alkyl, cyclohexyl, acryloxyethyl or methacryloxyethyl

X means —NH—, —NR— or —O—,

R<sub>1</sub> means a chemical bond, alkylene, alkylidene, SO<sub>2</sub>, O or S.

2. The color photographic material according to claim 1, wherein the compound of the formula II is used in the blue sensitive silver halide emulsion layer containing at least one yellow coupler in a quantity of 0.1 to 2 mol/mol of coupler.

3. The color photographic silver halide material according to claim 1, wherein the yellow coupler is a 2-equivalent pivaloyl coupler, the leaving group of which is attached to the coupling position either with oxygen or with nitrogen.

4. The color photographic silver halide material according to claim 1, wherein each of at least one blue-, green- and red-sensitive silver halide emulsion layers contain at least 80 mol % AgCl emulsions.

5. The color photographic silver halide material according to claim 1, which further contains at least one compound selected from the formulae (III), (IV) and (V) in a layer containing a color coupler,



in which

Y means a residue which is cleaved under chromogenic development conditions,

R<sup>31</sup> means alkyl, cycloalkyl, acylamino, sulphonamino, R<sup>32</sup>, R<sup>33</sup> and R<sup>34</sup> are the same or different and mean H, alkyl, cycloalkyl, hydroxy, acyloxy, alkoxy carbonyl, halogen, acylamino or carbamoyl,

R<sup>35</sup> means alkyl, cycloalkyl, alkoxy carbonyl, acylamino or carbamoyl or R<sup>31</sup> and R<sup>34</sup>, or R<sup>34</sup> and R<sup>35</sup>, or R<sup>35</sup> and R<sup>33</sup>, or R<sup>33</sup> and R<sup>32</sup> may form a 5- or 6-membered ring;



in which

R<sup>41</sup> means H, OH, alkoxy, aryloxy, acyl, acyloxy, alkyl or cycloalkyl,

R<sup>42</sup> and R<sup>43</sup> are the same or different and are H or alkyl, R<sup>44</sup> and R<sup>45</sup> are the same or different and are alkyl or cycloalkyl

Z means a group to complete a non-metallic 5- to 8-mem-

**27**

bered ring, wherein the R<sup>42</sup> and R<sup>45</sup>, R<sup>43</sup> and R<sup>44</sup>, R<sup>41</sup> and R<sup>44</sup> or R<sup>45</sup> may form a 5- to 8-membered ring,

R<sup>51</sup>—S—R<sup>52</sup>

(V)

in which

**28**

R<sup>51</sup> and R<sup>52</sup> are the same or different and are alkyl, cycloalkyl, aryl and the residues R<sup>51</sup> and R<sup>52</sup> may form a 5- to 8-membered ring.

\* \* \* \* \*